

# United States Patent Office

2,809,917

Patented Oct. 15, 1957

1

2,809,917

## SUSTAINED RELEASE PHARMACEUTICAL TABLETS

Victor M. Hermelin, University City, Mo.

No Drawing. Application October 17, 1955,  
Serial No. 541,031

6 Claims. (Cl. 167—82)

This invention relates in general to certain new and useful improvements in pharmaceutical preparations and, more particularly, to medicated granules which release the medication into the human system gradually over a sustained period of time and methods of making the same. This application is a continuation-in-part of my copending application Serial No. 461,354, filed October 11, 1954, now Pat. No. 2,736,682, which is, in turn, a continuation of an earlier application Serial No. 195,369, filed November 13, 1950, now abandoned.

It has been accepted practice in the compounding of pharmaceutical tablets to provide certain types of tablets with what has been commonly referred to as an enteric coating. The enteric coating is one which will resist the action of the gastric juices in the stomach and will not dissolve therein or be otherwise affected thereby so that the drug which is incorporated in the tablet will pass through the stomach and into the intestine. The so-called enteric coating is of such a nature that it will be dissolved very readily in the intestinal fluids so that the drug which has been enclosed in the enteric coating will become effective in the intestinal tract rather than in the stomach. Such tablets, however, are merely "delayed action" tablets. In other words, by selecting an enteric coating of the proper type and by using an appropriate amount, it is possible to delay the effective entry of the drug into the patient's system for a number of hours. The so-called "enteric coated" tablet is also used when it is desirable to introduce the medicament into the patient's intestinal tract without discharging any of the medicament into the stomach. These procedures are useful in certain applications, but the patient sooner or later receives the entire dosage in a single shot, so to speak.

Recently, efforts have been made to provide delayed dosage by surrounding an enteric coated core with a second layer or group of layers of medicament and then, largely for appearance, covering the resulting tablet, ellipsoid or sphere with a soluble sugar coating. The theory is that the sugar coating and outer layers dissolve in the stomach and almost immediately release the initial dosage which lasts the patient for several hours. Whereupon, the enteric coated core has reached the intestinal tract and dissolves therein very rapidly, releasing the second dosage. Even if this theory were borne out in practice, the net result would merely be a spaced interval "two shot" medication which is very little different in pathological effect from the simple business of giving the patient two smaller tablets at the same intervals. As a matter of fact, however, the existing methods of forming enteric coatings are not particularly accurate and the enteric coatings now in use are not always completely reliable. The research of Maney and Kuever (J. Am. Pharm. Soc. 30, 1941, p. 276), and of Abbott and Seepert (Pharm. J. 151, 1943, p. 52), suggests that various known enteric materials yield varying results and some such coatings seem to resist disintegration for periods up to five or six hours. Actual tests with various types of

2

enteric coatings using the in vitro method of Maney and Kuever have shown that most available enteric coatings dissolved to an appreciable extent in the gastric juices of the stomach or at least are attacked by such gastric juices to such an extent as to lose physical or structural strength, a factor which has been hitherto overlooked. In the stomach, peristaltic action is severe enough to disrupt the physically weakened enteric coating and the drug or medicament enters the system with a surge, as has been discovered by blood level studies. The important point, however, is that enteric coatings, however efficient or inefficient they may be, merely withhold the medicament for some "time-delay" period and then release it to the patient's system in the same "surge dose" as though the period of time delay had not occurred. In other words, the patient ultimately gets the surge.

However, recent pharmacological investigations have shown that with many drugs the patient responds far better to sustained minute-incremental dosage, that is to say, very minute quantities administered at very short intervals continuously over sustained periods of time. This can be referred to, for want of a better term, as the "trickle system." Such procedures have been recognized for quite some time with respect to liquid medications such as the trickle treatment with penicillin for syphilis. The use of conventional enteric coated tablets, however, for the reason heretofore set out will not achieve even an approximation of sustained minute-incremental dosage.

It is the primary object of the present invention, therefore, to provide a pharmaceutical preparation having a unique and novel composition and structure, which, as a result of a drug or medicament, can be administered in a persistent sustained incremental dosage.

It is also an object of the present invention to provide a pharmaceutical preparation which is capable of maintaining a desired level of medication within the patient's system over prolonged periods of time.

It is a further object of the present invention to provide a pharmaceutical preparation which has a unique and novel composition and structure, which is simple and precise in its action and which is economical to produce.

It is also an object of the present invention to provide methods of making pharmaceutical preparations of the type stated.

With the above and other objects in view, my invention resides in the novel features of form, construction, arrangement, and combination of parts presently described and pointed out in the claims.

Broadly speaking, the present invention resides in the discovery that a pharmaceutical preparation adapted for sustained minute-incremental dosage can be made by intimately mixing various enteric water insoluble excipients, such as shellac, with powdered drugs to form a somewhat pasty mass which is then spread on drying trays and dried to produce a rough granular material. This granular material is crushed and remixed with the excipient to form a pasty mass which is then spread on trays and dried again to form a rough granular material. This procedure of crushing, mixing with excipient, and tray-drying is repeated a number of times and finally the end product is screened to produce a granule of substantially uniform size. It has been found that the excipient and the medicament are intimately mixed or dispersed throughout the mass of each granule in the form of very minute particles. Visual examination of the granules under high-magnification shows that the surface thereof is not covered with a continuous film of the dried excipient or a continuous film of the medicament, but, rather, is dotted with minute particles of the dried excipient and minute particles of the medicament in a sort of heterogeneous arrangement. Furthermore, this general physical

structure exists throughout the granule. By both in vitro tests and blood-level studies, it clearly appears that these granules, when in the human stomach and intestinal tract are neither soluble or insoluble in the strictest sense of these terms, but, instead, the medicament leaches out steadily in minute increments or doses, that is to say, as a sustained "trickle."

This material, however, for many types of illnesses, may not release a sufficient amount of the drug or medicament initially to build up to the desired blood-level concentration. Therefore, it is necessary to provide some means by which an initial surge does can be conveniently given. It has been found that this can be accomplished by forming a unique type of laminated tablet, that is to say, a tablet which in effect consists of two identically shaped cylindrical slugs adhered together in back-to-back relation. To make such a laminated tablet, a tableting machine of conventional type is used having a series of die-cavities and reciprocating punches. The cams of the machine are set so that each punch will enter its companion die-cavity twice before the tablet is ejected. The machine should also be provided with two conventional feeding hoppers located at spaced positions along the path of movement of the die plate. Each die-cavity is initially filled with a suitable quantity of the granules prepared as above described and the punch driven into the die recess to compress the granules. The punch, upon being withdrawn, leaves the die-cavity about half-filled. Then a quantity of plain drug, i. e. not formed into slow-release granules, is charged into the unfilled portion of the die-cavity. The punch is again driven into the die-cavity, compressing the second filling and the whole tablet into a firm two-ply or laminated tablet.

While this invention is not intended to be limited thereby, the following are examples of pharmaceutical preparations which can be made in accordance with the present invention:

*Example I*

3 lbs. of dicalcium phosphate and 1 lb. d-amphetamine sulfate is mixed in the dry. To this mixture, wax-free shellac (3 lb. cut-U. S. P. grade) is slowly added with agitation and in sufficient amount to produce a pasty mass which is spread out on cloth drying trays and air dried for 7-10 hours. The resulting product, when removed from the drying trays, forms a free flowing granular mass in which the granules have an average size of wheat grains. These granules are then crushed to about the size of coarse sugar and again mixed with enough shellac (of the type above) until a pasty mass results. This mass is again placed on cloth drying trays and the above procedure repeated for a total of eleven times, using a total of about 1 gallon of shellac. The first four mixing-drying steps are repeated over a time cycle which involves about 7 to 10 hour drying periods and all subsequent mixing-drying steps include about 20 to 22 hour drying periods. These time periods can be speeded up by placing the drying trays in a hot room. The hot room should be maintained at about 100° to 120° F. with a relative humidity not in excess of 30% and the material dried until the granules are hard and frangible, that is to say, will form fine-grained particles upon crushing. Final yield is approximately 15 lbs. of granules of heterogeneous and irregular shapes.

Upon assay, the granules are precisely uniform in constituency. In other words, any given weight of granules will be found to contain the same dosage of amphetamine. Of course, each batch should be assayed and the actual amphetamine content by weight or percentage determined. It has been found that by following a standardized manufacturing procedure, successive batches of granules have closely similar assays well within admissible limits of pharmaceutical accuracy. However, this is not overly important since the granules thus formed are measured into capsules or tableted by conventional procedure for administration to the patient and any variations in con-

tent can be taken into account in making up the capsule or tablet.

These slow-release granules are then formed into a two-ply or laminated tablet with plain or untreated 5 amphetamine sulfate in the initial-dosage portion as above described.

*Example II*

A dry mixture of 12 oz. d-amphetamine sulfate, 8 oz. 10 secobarbital and 3 lbs. 8 oz. dicalcium phosphate is taken up with shellac as per Example I employing approximately 1 gal. shellac in eleven successive mixing-drying steps. Yield approximately 16 lbs. of granules.

These slow-release granules are then formed into a 15 two-ply or laminated tablet with plain or untreated amphetamine sulfate in the initial-dosage portion as above described.

*Example III*

A dry mixture of 2 lbs. pentobarbital, 1 lb. 20 phenobarbital and 6 oz. d-amphetamine sulfate, 3 lbs. dicalcium phosphate is taken up in shellac as per Example I employing nine successive mixing-drying steps.

These slow release granules are then formed into a 25 two-ply or laminated tablet with a plain or untreated mixture of pentobarbital, d-amphetamine sulfate, and dicalcium phosphate in the above named proportions in the initial-dosage portion, as above described.

The above described procedure has been employed in 30 making granules with a wide variety of drugs or medicinals, such as, for instance, scopolamine, methyl bromide, pentaerythritol tetranitrate, sodium nitrite, hexamethonium chloride, veratrum viride, reserpine, stilbesterol, methyl testosterone, phenobarbital, pyralimine, digitoxin, and Caffeine. In each instance, the quantity of the drug is calculated by usual arithmetic methods well known in pharmaceutical manufacturing.

It has also been found that other liquid excipients, such 35 as a mixture of castor oil, stearic acid, and confectioner's glaze (i. e. shellac) can be employed in practicing the herein described invention. Similarly, by increasing the number of mixing-drying steps, it is possible to slow down the rate of entry of the drug into the patient's system and, conversely, by lowering the number of successive mixing-drying steps, it is possible to speed up the rate of entry 45 of the drug into the patient's system. However, it has been found that a minimum of such steps is two and a practical maximum is fifteen, since additional mixing-drying steps resulting in such a slow rate of drug absorption by the patient has been found to be impractical for 50 presently known medical purposes.

It should be understood that changes and modifications in the form, construction, arrangement, and combination of the several parts of the pharmaceutical preparation may 55 be made and substituted for those herein shown and described without departing from the nature and principle of my invention.

Having thus described my invention, what I claim and desire to secure by Letters Patent is:

1. The method of making a laminated tablet having a 60 layer containing an immediate release medicated preparation and a layer containing a delayed release medicated preparation having a slow but continuous and attenuated solubility in the gastro-intestinal tract, which method comprises intimately mixing a powdered drug and an enteric water insoluble excipient to produce a pasty mass, drying the mass slowly without agitation in such a manner as to produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to

granular particles, said second mixing, drying and crushing operations constituting a second cycle, said process consisting of not less than three nor more than fifteen mixing, crushing and drying cycles repeated in successive order whereby to produce the delayed release medicated preparation, introducing one of said medicated preparations into a die cavity and compressing same to form a first solid layer, introducing the other of said preparations into the cavity on top of the compressed first preparation, and thereafter compressing said other preparation into a second solid layer which adheres firmly to said first solid layer.

2. A method in accordance with claim 1 wherein the enteric water insoluble excipient is shellac.

3. A method in accordance with claim 1 wherein the enteric water insoluble excipient comprises a mixture of shellac and stearic acid.

4. A pharmaceutical preparation comprising a single tablet having two laminated layers attached integrally to each other, one layer containing a medicated preparation in readily assimilable form for immediate release into a patient's system and the other layer containing a medicated preparation having a slow but continuous and attenuated solubility in the gastro-intestinal tract, said last-mentioned preparation containing a solid mass of dry discrete granules, each said granule being made by intimately mixing a powdered drug and an enteric water insoluble excipient to produce a pasty mass, drying the mass slowly without agitation in such a manner as to

produce a rough granular material, breaking up the rough granular material by light crushing, whereby to reduce it to granular particles, said mixing, drying and crushing operations constituting one cycle, and remixing the granular particles with an additional quantity of the excipient to produce a pasty mass, redrying such pasty mass slowly and without agitation in such a manner as to produce a granular material, again breaking up the rough granular material by light crushing, whereby to reduce it again to granular particles, said second mixing, drying and crushing operations constituting a second cycle, said process consisting of not less than three nor more than fifteen mixing, crushing and drying cycles repeated in successive order.

5. A pharmaceutical preparation in accordance with claim 4 wherein the enteric water insoluble excipient is shellac.

6. A pharmaceutical preparation in accordance with claim 4 wherein the enteric water insoluble excipient comprises a mixture of shellac and stearic acid.

#### References Cited in the file of this patent

#### UNITED STATES PATENTS

|    |           |          |               |
|----|-----------|----------|---------------|
| 25 | 701,438   | Whyte    | June 3, 1902  |
|    | 2,052,376 | Zellers  | Aug. 25, 1936 |
|    | 2,736,682 | Hermelin | Feb. 28, 1956 |

#### OTHER REFERENCES

Clarkson: Tablet Coating (New York, 1951), p. 61.